

Jan. 22, 1952

H. D. HARTOUGH ET AL

2,583,509

SOLVENTS CONTAINING NITRILES

Filed Oct. 16, 1947

2 SHEETS—SHEET 1

FIG. 1



FIG. 2



INVENTOR.

HOWARD D. HARTOUGH  
BY HOWARD W. SHELDON

*Francis F. Johnston*  
AGENT OR ATTORNEY

Jan. 22, 1952

H. D. HARTOUGH ET AL

2,583,509

SOLVENTS CONTAINING NITRILES

Filed Oct. 16, 1947

2 SHEETS—SHEET 2

FIG. 3



FIG. 4



INVENTOR.

HOWARD D. HARTOUGH  
BY HOWARD W. SHELDON

*Francis Johnston*

AGENT OR ATTORNEY

## UNITED STATES PATENT OFFICE

2,583,509

## SOLVENTS CONTAINING NITRILES

Howard D. Hartough, Pitman, and Howard W. Sheldon, Woodbury, N. J., assignors to Socony-Vacuum Oil Company, Incorporated, a corporation of New York

Application October 16, 1947; Serial No. 780,208

## 1 Claim. (Cl. 106—311)

The present invention relates to solvents for natural and synthetic resins, gums, etc. and, more particularly, to composite solvents of more than linear kauri-butanol number.

As pointed out by W. J. Sweeney and J. A. Tilton in Industrial and Engineering Chemistry for June 1934, "The widespread use of synthetic resins—for example the phenolformaldehyde and the alkyd, or Glyptal types"—has created demands for naphthas of higher solvency than the common run of petroleum solvents marketed in the past. While the coal-tar solvents such as toluene and high-flash naphtha possess high solvency powers, they have certain objectionable properties, in particular poor odor.

The gum kauri-butanol test is frequently utilized by both the oil refiner and the trade for evaluating solvent naphthas. This test consists essentially of titrating 20 grams of a standard gum kauri solution (100 grams of gum kauri dissolved in 500 grams of n-butanol) in a 200 centimeter Ehrlemeyer flask with the solvent to be tested. The end point is reached when the normally clear liquid acquires a slight turbidity. This is determined by placing a printed page (10-point print) beneath the flask and noting when the print, as viewed through the solution, just becomes blurred. The number of cubic centimeters of solvent required to produce this end point is called the "kauri-butanol value" of the solvent.

It has now been discovered that the kauri-butanol values of solvents can be enhanced in more than a linear proportion by combining recognized solvents with aromatic nitriles. This is surprising since it is to be expected that a mixture of two solvents would have a kauri-butanol value closely approximating the weighted average of the kauri-butanol values of the solvent and the aromatic nitrile. For example, the kauri-butanol value for benzene is 103 and that for benzonitrile is 122. It would be expected that a blend containing 50 volume per cent of each would have a kauri-butanol value of 115. However, a blend containing 50 volume per cent of benzene and 50 volume per cent of benzonitrile has a kauri-butanol value of 139. Accordingly, it is an object of the present invention to provide a multicomponent solvent having a kauri-butanol value greater than the calculated weighted average kauri-butanol value for the components. It is another object of the present invention to provide multicomponent solvents containing an amount of an organic nitrile effective to produce a kauri-butanol value for the multicom-

ponent solvent greater than the calculated weighted average of the kauri-butanol values of the components. Other objects and advantages will become apparent to those skilled in the art from the following description taken in conjunction with the drawings in which:

Figure 1 is a graph of the observed and calculated kauri-butanol values for various mixtures of benzene and benzonitrile;

Figure 2 is a graph of the observed and calculated kauri-butanol values for various mixtures of n-hexane and benzonitrile;

Figure 3 is a graph of the observed and calculated kauri-butanol values for various mixtures of benzonitrile and an aromatic petroleum stock having a boiling range of 275 degrees to 375 degrees Fahrenheit and comprising a mixture of polyalkyl benzenes, paraffins and naphthenes, the polyalkyl benzenes being predominantly dimethyl benzenes; and

Figure 4 is a graph of observed and calculated kauri-butanol values for various mixtures of benzonitrile and an intermediate petroleum naphtha having a boiling range of 190 to 314 degrees Fahrenheit, an aniline number of 63 degrees Fahrenheit and a kauri-butanol value of 36.

Those skilled in the art will immediately recognize that the curves for relatively pure aromatic solvents mixed with benzonitrile and for an aromatic solvent containing, say 30 per cent, non-aromatic hydrocarbons mixed with benzonitrile have a slope for amounts of benzonitrile up to 50 volume per cent different than the slopes of curves for mixtures of aliphatic or predominantly aliphatic solvents and up to 50 volume per cent of benzonitrile. Thus, for example, the kauri-butanol value for a 90 volume per cent benzene—10 volume per cent benzonitrile mixture is 125 while the calculated value is 105. This represents an increase of 19 per cent of the calculated kauri-butanol value. Similarly, the observed kauri-butanol value for a 90 volume per cent aromatic petroleum stock—10 volume per cent benzonitrile mixture is 98 while the calculated value is 83 or an increase of 18 per cent. On the other hand, the observed kauri-butanol value for a 90 volume per cent intermediate naphtha—10 volume per cent benzonitrile mixture is 48 while the calculated value is 45; an increase of about 7 per cent. Similarly, the calculated kauri-butanol value for a 90 volume per cent n-hexane—10 volume per cent benzonitrile mixture is 36 and the observed value is 36. The following table provides a comparison of the effect of adding varying amounts

of benzonitrile, an aromatic nitrile to various solvents.

butanol value of the mixture being the sum of the kauri-butanol values of each component

| Vol. Per Cent Benzonitrile | Vol. Per Cent Solvent | Benzene, kauri-butanol value |      |               | Aromatic petroleum stock, kauri-butanol value |      |               | Intermediate naptha, kauri-butanol value |      |               | n-hexane, kauri-butanol value |      |               |
|----------------------------|-----------------------|------------------------------|------|---------------|-----------------------------------------------|------|---------------|------------------------------------------|------|---------------|-------------------------------|------|---------------|
|                            |                       | obs.                         | cal. | Per cent inc. | obs.                                          | cal. | Per cent inc. | obs.                                     | cal. | Per cent inc. | obs.                          | cal. | Per cent inc. |
| 0                          | 100                   | 103                          | 103  | 11.7          | 79                                            | 80   | 3.7           | 36                                       | 39   | -----         | 28                            | 29   | -----         |
| 2                          | 98                    | 115                          | 104  | 15.4          | 83                                            | 81   | 8.6           | 40                                       | 40   | -----         | 29                            | 31   | -----         |
| 5                          | 95                    | 120                          | 104  | 19.0          | 99                                            | 83   | 19.3          | 48                                       | 45   | 6.7           | 36                            | 36   | -----         |
| 10                         | 90                    | 125                          | 105  | 22.2          | 115                                           | 88   | 30.7          | 66                                       | 54   | 22.2          | 50                            | 45   | 11.1          |
| 20                         | 80                    | 132                          | 107  | 23.2          | 128                                           | 92   | 39.2          | 88                                       | 62   | 25.8          | 75                            | 55   | 36.4          |
| 30                         | 70                    | 135                          | 109  | 18.2          | 137                                           | 96   | 42.7          | 108                                      | 70   | 54.3          | 100                           | 65   | 53.9          |
| 40                         | 60                    | 138                          | 111  | 23.2          | 142                                           | 100  | 42.0          | 127                                      | 80   | 58.8          | 118                           | 74   | 59.5          |
| 50                         | 50                    | 139                          | 112  | 20.8          | 144                                           | 108  | 33.3          | 139                                      | 88   | 57.3          | 133                           | 83   | 60.3          |
| 60                         | 40                    | 138                          | 114  | 21.0          | 141                                           | 109  | 29.4          | 145                                      | 96   | 51.0          | 140                           | 93   | 50.5          |
| 70                         | 30                    | 137                          | 116  | 18.1          | 136                                           | 113  | 20.4          | 145                                      | 105  | 38.1          | 141                           | 102  | 38.3          |
| 80                         | 20                    | 133                          | 118  | 12.7          | 129                                           | 117  | 10.3          | 140                                      | 114  | 22.8          | 136                           | 112  | 21.4          |
| 90                         | 10                    | 130                          | 120  | 8.3           | 122                                           | 122  | -----         | 122                                      | 122  | -----         | 122                           | 122  | -----         |
| 100                        | 0                     | 122                          | 122  | -----         | 122                                           | 122  | -----         | 122                                      | 122  | -----         | 122                           | 122  | -----         |

The data presented in the table together with the graphs of Figures 1 to 4 establish that for non-aromatic or predominantly non-aromatic solvents the minimum amount of added aromatic nitrile to produce a practical increase in the kauri-butanol value is about 20 volume per cent. However, for aromatic or predominantly aromatic solvents the minimum amount of added aromatic nitrile to produce a practical increase in the kauri-butanol value is about 2 to about 10 volume per cent. Accordingly, the minimum effective concentration of aromatic nitrile in the multicomponent solvent is about 2 volume per cent when the basic solvent is predominantly aromatic in nature and about 20 volume per cent when the basic solvent is predominantly non-aromatic in nature. It is also to be noted that concentrations of aromatic nitrile in excess of about 70 volume per cent of the total multicomponent solvent are ineffective to produce enhanced kauri-butanol values when the basic solvent is predominantly aromatic in character whereas concentrations as high as 80 volume per cent of the multicomponent solvent are effective to produce enhanced kauri-butanol values when the basic solvent is predominantly non-aromatic in character. Thus, the novel multicomponent solvent comprises an aromatic nitrile and one or more hydrocarbons, the mixture containing a concentration of aromatic nitrile effective to produce kauri-butanol values at least 10 per cent greater than the calculated kauri-butanol value of the mixture, the calculated kauri-

20 multiplied by the volume per cent of said component in the multicomponent solvent.

We claim:

25 A multicomponent solvent for resins, gums, and the like which consists essentially of a predominantly aromatic hydrocarbon solvent for resins, gums, and the like and benzonitrile, said benzonitrile being present in said multicomponent solvent in a concentration of about 10 to about 80 volume per cent, said concentration of benzonitrile being sufficient to produce a multicomponent solvent having a kauri-butanol value greater than the calculated kauri-butanol value of said mixture.

30 HOWARD D. HARTOUGH.

HOWARD W. SHELDON.

#### REFERENCES CITED

35 The following references are of record in the file of this patent:

#### UNITED STATES PATENTS

| Number    | Name          | Date          |
|-----------|---------------|---------------|
| 2,388,082 | Roediger      | Oct. 30, 1945 |
| 2,450,639 | Denton et al. | Oct. 5, 1948  |
| 2,508,215 | Bishop        | May 16, 1950  |

#### OTHER REFERENCES

Journal of Chemical Society, Article by Martin and Collie, pp. 2658-65 (1932).

Journal American Chemical Society, vol 24, 1902, Bozert and Hand, pp. 1031-1032.